

Aug. 6, 1968

C. E. PENOYER

3,396,181

SUPERBODIED OILS

Filed Oct. 13, 1965

2 Sheets-Sheet 1



Fig. I

INVENTOR  
CHARLES E. PENOYER  
BY *Kramer & Stenger*

ATTORNEYS.

Aug. 6, 1968

C. E. PENOYER  
SUPERBODIED OILS

3,396,181

Filed Oct. 13, 1965

2 Sheets-Sheet 2



1

3,396,181

**SUPERBODIED OILS**

Charles E. Penoyer, Chagrin Falls, Ohio, assignor to The Sherwin-Williams Company, Cleveland, Ohio, a corporation of Ohio

Filed Oct. 13, 1965, Ser. No. 495,596  
7 Claims. (Cl. 260—407)

**ABSTRACT OF THE DISCLOSURE**

There is provided an improved process for superbodying unsaturated fatty oils to produce a product which is free from gelled particles and false body and having a viscosity in the range of from 20 minutes to 75 minutes, Gardner-Holdt. The process is characterized by first thermally bodying the oil by causing it to polymerize under the influence of heat, and finally subjecting the oil in bulk form to oxidative polymerization.

This invention relates to extraordinarily high viscosity oils derived from unsaturated fatty oils, particularly drying oils of the natural or synthetic types, which oils are characterized by freedom from gel particles and "false body." More particularly, the present invention relates to the method for producing oxidized superbodied oils having viscosities in the range of from about 20 minutes to about 75 minutes, Gardner-Holdt, herein characterized as "superbodied oils." All viscosities referred to herein are Gardner-Holdt unless specifically otherwise indicated. It is to be understood that the viscosity value referred to herein is based upon the time required for an air bubble to travel the length of a standard Gardner varnish viscosity tube under standard temperature conditions (77° F.).

This invention is an improvement upon the process of my copending application Ser. No. 329,197, filed Dec. 9, 1963, now U.S. Patent No. 3,337,593, which application was in turn an improvement upon the invention of James A. Arvin described and claimed in Patent No. 2,607,784.

It has been found that unsaturated fatty oils (unsaturated fatty acid polyesters) when bodied at atmospheric pressure to the point of incipient gelation and thereafter blown with steam to a high body, e.g., one hour or more, develops a gel structure which is detrimental in coating compositions. False body is another difficulty attendant superbodied oils. This "false body" is believed to be due to the presence of intramolecular attraction forces (Van der Waals forces) which upon dilution with a thinner, solvent, or other additive, e.g., fatty acid or rosin, are dissipated with the result that the viscosity, or body, of the oil decreases more than is accountable to the dilution effect of the added material. Durability of the film is related to the actual body of the oil, and when an oil exhibits "false body" this relationship is destroyed and it is not possible to estimate the durability on the basis of viscosity. However, when the oil possesses a true body in the range of from 20 to 75 minutes, which body results from the development of intermolecular carbon-carbon bonds through polymerization of the mass, then the relationship of durability to oil body is such as to enable estimation of the durability of a coating composition containing such oil to a much better degree.

The procedure of the invention varies from that described and claimed in the aforementioned Arvin patent in several important respects. First, the bodying operation hereof is carried out under vacuum instead of at atmospheric pressure. Secondly, according to the improved process, moisture is introduced into the bulk of the oil from and after arrival at the point of incipient polymeri-

2

zation instead of from and after arrival at the point of incipient gelation, and continued in the process until the desired body is reached. When these changes are made in the Arvin process, there results a bodied oil which is free of gel particles, or nuclei, which interfere with the later processing of coating compositions and the shelf-life of the product. Moreover, these products are characterized by true body as distinguished from "false body."

As indicated above, there is a relationship between viscosity and the durability of a coating composition containing a highly bodied oil having a true body or viscosity in the range of from 20 minutes to 75 minutes. Although I do not wish to be bound to any theory for explaining such relationship, it is believed that in a normal oil of the drying type when applied as a paint film, most of the hardening is brought about by reaction of the oil with oxygen, i.e., oxidative polymerization. Even in those cases where partially bodied oils are utilized as the binder, or vehicles, for the pigment, the major portion of the hardening reaction is brought about by cross-linking of the molecules with oxygen. The predominance of oxidative polymerization in the process of film solidification yields a product which is subject to decomposition, e.g., on exposure to actinic light, which leads to degradation of the film. Oxidative products of polymerization are more susceptible to deterioration than condensation products having carbon-to-carbon bonds. To increase the ratio of the more stable carbon-to-carbon bonding in the final solidified products with a corresponding reduction in the amount of oxidative polymerization which is permitted to take place, it has become the practice to body the oils by heating, or by means of a catalyst. Such bodied oils may be cut with a thinner to a suitable viscosity, and when applied and the thinner removed by vaporization, the resultant coating composition film is well along the way to solidification due to the preliminary carbon-to-carbon polymerization. The limit of prebodying oils has heretofore been determined by the occurrence of gelation in the course of such processes and the difficulty of applying protective coatings based thereon. The presence of gel particles within the bulk of the oil seemed to promote further solidification or gelation of the mass prior to application and hence instability of the product on the shelf. The presence of such particles initiates the gelation reaction.

The present invention is an extension of that which has already been disclosed in the aforementioned Ser. No. 329,197, and to two other applications filed concurrently therewith bearing Ser. Nos. 329,191, now U.S. Patent No. 3,333,975, and 329,196, now U.S. Patent No. 3,333,976. The invention involves the pre-oxidation of the highly heat polymerized oils in bulk under controlled conditions until a certain higher viscosity or range of higher viscosity is achieved through a pre-oxidative process. This is distinct from film oxidation, or post application oxidation in a film. The resultant product has very distinct advantages in water emulsion paints. Drying throughout the film is achieved much more rapidly. To illustrate, the oxidized superbodied oil and the unoxidized superbodied oil, both with 0.139% cobalt naphthenate drier, and deposited from solvent solutions drawn down upon glass to leave a .003" wet film, and dried at 50% relative humidity, at 81° F., showed respectively, set-to-touch times of 58 minutes and 168 minutes, and dry-to-touch times of 98 minutes and 198 minutes. Thus, after pre-oxidizing the superbodied oil the set-to-touch time is only 35% of the time required by the original superbodied oil. The oxidized superbodied oil dries-to-touch in 50% of the time required by the unoxidized superbodied oil. Similar results were obtained when these oils were deposited in

water emulsion form as films of ".003" wet thickness, dried at 55% relative humidity, and 83° F.

Secondly, there is obtained a higher solvent-reduced oil viscosity of the pre-oxidized superbodied oil which enables, through a greater structural rigidity, a greater resistance to rain by the paint film in the very early period immediately following its formation. By actual example, the solvent reduced oil viscosity of the superbodied oil is about 1 minute and 50 seconds for the unoxidized oil, compared with approximately 3 minutes and 50 seconds for the oxidized oil. It has been found that it is not feasible to provide the increased viscosity through more extensive heat polymerization or thermal polymerization since the reaction cannot be controlled in production operations well enough to avoid gelation of the oil, or to avoid an uneconomical extension of the time of processing.

Third, the pre-oxidation treatment and the ensuing higher viscosity reduces any tendency for unsightly flashing of the paint into shiny areas after the lap from brush burnishing again because the structural rigidity is higher and there is, therefore, less tendency of the more viscous oil to flow under the smearing action of the brush bristles over otherwise uncoated pigment surfaces to raise the gloss or sheen of the paint in the area immediately after the lap.

It has also been found that there is an improvement in the emulsion stability as a result of the higher viscosity of the oil and the consequent lesser tendency for the emulsion internal phase droplets to flow together and coalesce. Still further because of the strong drying powers of the pre-oxidized superbodied oil as compared with the unoxidized superbodied oil, it is practical to include in the emulsion formula larger quantities of surfactants and protective colloids, which frequently tend to interfere with the drying process.

The resulting advantage of permissible larger contents of emulsifiers and protective materials is greater emulsion stability through dispersion of the oil into an extremely fine particle size internal phase. Attendant advantages of improved emulsion stability and the smaller particle size include increased paint package stability, improved weathering durability, retention of tinting colors, and more pleasing low angular sheen of the dried film.

Briefly, the departure from the procedure set forth in the foregoing copending Ser. Nos. 329,191, 329,196 and 329,197 is that prior to the reduction of the oil with the solvent, the temperature is brought to a level of about 150° F. to 200° F., preferably from 170° F. to 180° F., and the viscosity of the superbodied oil is reduced with a solvent to from about 2 minutes to about 10 minutes, preferably from about 3 minutes to about 5 minutes. This thinned oil is then subjected to mechanical agitation in a tank equipped with steam-heating or water-cooling coil and a perforated coil for passing air into and through the oil while mechanically agitating it to further break up the air bubbles and to lengthen the path of travel by the air, all in the interest of creating a more extensive oil-air interface. The aeration is conducted at this temperature for a period of from about 25 hours to about 60 hours preferably from 30 to 40 hours, or until the viscosity of the solvent-free oil is in the range of from 20 minutes to 75 minutes. The oil becomes free of solvent during the early stages of the blowing operation by evaporation aided by the flow of the oxygen containing gas through the oil.

In general, the method of making a superbodied unsaturated fatty oil free from gel particles and false body and having a viscosity in the range of from 20 minutes to about 75 minutes, comprises the steps of heating the body of the oil under subatmospheric pressure to the temperature of incipient polymerization, i.e., the temperature at which any increase in temperature causes a significant or practicable increase in the body, or viscosity, of the oil. Generally, this temperature is in the neighborhood of from about 475° F. to about 525° F., and may be spe-

cifically predetermined in the laboratory for any oil. At or just below this point, the bulk of oil is brought into contact with water vapor, for example by the introduction of water, or steam, into the hot body of oil. Thereafter, the temperature of the oil is increased to initiate and sustain polymerization of the oil, i.e., bodying of the oil while continuously contacting the oil with water vapor. Heat induced polymerization of the oil is continued to a maximum temperature of about 615° F. for a period of time sufficient to increase the viscosity of the oil to from 20 minutes to about 75 minutes, while continuously contacting the body of oil with water vapor. When the viscosity has been determined to be at the desired point by periodic sampling, or by prior determination of the required amount of time to reach a desired body at a given temperature, the contacting of the body of oil with moisture is discontinued. Therefore, the thermal polymerization reaction is "checked" by suddenly dropping the temperature to below the temperature of further polymerization of the oil. "Checking" is a term of art for arresting polymerization and is achieved by rapid reduction of the temperature of the batch to a temperature below which further polymerization will not occur. This is usually below about 475° F.

The annexed drawing diagrammatically illustrates commercial size apparatus for making oxidized superbodied oils in accordance herewith. While the thermal bodying procedure of the present invention can be carried out in the absence of a catalyst, it has been found for certain purposes to be highly desirable to include an oil-soluble alkali metal salt or alkaline earth metal salt of a high molecular weight aliphatic acid or cycloaliphatic acid, either saturated or unsaturated. The presence of a catalytic amount, i.e., 0.1% to about 2% by weight of the oil of such a material has been found to confer several important properties on the nature of the reaction and on the final product both of which can be utilized with advantage. The presence of such metallic salts in such low amount in the oil, alone or in combination with a lead salt of a similar acid material and also soluble in the oil, has been found to cause a desirable increase in the amount of hydroxyl bearing components in the final oil. This effect is one principally of promoting esterifications and especially the formation of hydroxyl-bearing partial esters. Some aid to the quality of the final product accrues through the addition of polyols for additional partial ester formations. The lead salt may also be alone for this purpose but with a somewhat lower degree of effectiveness. Increased hydroxyl content, as hereinafter more particularly pointed out renders such oil highly useful in the production of oil-in-water emulsions from such high viscosity oils. Thus, there may be used the sodium, potassium, lithium, calcium, magnesium, barium, strontium and lead salts or mixtures of such salts, of high molecular weight aliphatic, saturated or unsaturated, fatty acids containing from 10 to 22 carbon atoms or more, and including cycloaliphatic acidic materials; such as, isodecanoic, dodecanoic, ricinoleic, stearic, oleic, linoleic, linolenic, naphthenic acid, rosin acids, dimer fatty acids, e.g. dimerized linseed oil fatty acids, etc. When a lead soap is used alone or in conjunction with the alkali or alkaline earth metal soap, it is present in an amount generally in the range of from about 0.05% to about 2% by weight of the oil. The lead soap, if used with a co-operating soap, may be added along with the co-operating soap or at a different time in the bodying cycle. It has also been found that suitable salt materials of this character soluble or dispersible in the oil may be formed in situ by adding to the polymerization batch an oxide of the metal, for example calcium oxide, magnesium oxide, barium oxide, lead oxide, or a carbonate, e.g. calcium carbonate. Increase in the organic hydroxyl content of the final oil is readily ascertained from infrared analysis of the final product. With respect to the salt additions, it is the presence of the metallic moiety in a form soluble or dispersi-

ble in the oil rather than the specific nature of the organic acid moiety which is important.

It becomes convenient at this point to illustrate the process of the present invention in considerable detail by giving a specific example of the production of a bodied vegetable drying oil made from an alkali refined commercially available linseed oil material. While it is desirable that the base oil be of high quality as represented by an alkali refined, bleached and refrigerated product, raw linseed oil may be used. In any case, the starting material should be without a tendency upon heating a high temperature such as 585° F., especially in the presence of steam, to precipitate solid substances. Raw vegetable oils should be conditioned prior to and/or in the bodying process that they do not precipitate or "break out" solid substances commonly contained in these oils. The processes for such conditioning are well known in the art. The base oil should preferably have, but not necessarily so, a low free fatty acid content and a light color. Any of the common drying oil materials alone or in combination with each other, and including long oil modified synthetic resins as long oil modified alkyd resins, etc. may be used. Thus, linseed oil, dehydrated castor oil, soybean oil, safflower oil, tung oil, perilla oil and mixtures of such oils may be used as well as the corresponding oil modified alkyd and polyester type resinous materials. Copolymerized drying oils including styrenated drying oils, e.g. styrenated linseed oil, which oils are well known in the art, may also be used in accordance with this process.

Utilizing an apparatus such as diagrammatically shown in the annexed drawing, and with alkali refined, bleached and refrigerated linseed oil as an example, 3700 pounds of this oil is heated in a varnish kettle while mechanically agitating under a vacuum of at least about 24" of mercury to a temperature just below that where significant polymerization takes place, e.g. 450° F. At this point, the mass has arrived at incipient polymerization and further increase in temperature causes polymerization and an increase in viscosity. It is preferred that carbon dioxide, or nitrogen or other inert gas be passed through the linseed oil during the heating from the starting temperature (room temperature) to about 450° F. When the temperature has reached 450° F. just prior to the onset of homopolymerization which causes an increase in viscosity, it is preferable to substitute steam for part or all of the carbon dioxide or other inert gas. The application of steam to the body of oil may be through a conventional bubble ring, or by mere introduction through pipes located at the bottom of the container. The flow of steam through the entire mass of oil is maintained throughout the remainder of the polymerization operation. During the last half hour of the operation, it may be found desirable that an inert gas such as carbon dioxide or nitrogen be substituted for the steam again to provide a purging of the oil of any substantial amount of residual moisture.

The temperature of the oil is increased while the application of steam is continued until a bodying temperature of about 575° F. is reached. The mechanical agitation and steaming are continued as the bodying temperature is maintained until a viscosity of about 45 seconds is achieved at which point the vacuum is temporarily released, and about 0.29% by weight of the original oil of a mineral spirits solution of lead isodecanoate containing 24% lead, and 0.44% by weight of lithium naphthenate, containing 1.4% lithium, are added. The addition is not absolutely required for the operation of this process, but it has been found advantageous in that it aids the development of emulsifiability of the final product. In general, the amount of alkali metal or alkaline earth metal added as a soap soluble or dispersible in the oil is generally from about 0.002% to about 0.010% by weight of the oil, when calculated as the metal.

The conditions of bodying are maintained as above described until a viscosity of approximately 12 minutes is

reached. This viscosity marks a stage in the bodying process where operating temperatures are desirably dropped to lower levels and extreme care taken to avoid excessive local overheating. Excessive local overheating has been found, despite the steam treatment, to promote the formation of irreversible gel particles. Accordingly, it is recommended practice that at this point of viscosity development to drop the temperature, for example, from about 580° F. to from about 545° F. to 560° F. At this point, the mass has a viscosity of about 20 minutes, and the elapsed time in reducing the temperature of the mass has been about 30 minutes. The temperature of the batch is then allowed to drift slowly downward until ultimately a temperature of only about 470° F. is reached and the final viscosity is about 52 minutes. At this point, the batch is suddenly cooled to about 450° F. using a water in a coil immersed in the oil or any other suitable cooling means. Upon reaching the temperature of about 450° F., the pressure upon the batch is increased to atmospheric, and the entire quantity of bodied linseed oil is pumped in about 5 minutes elapsed time to a predetermined quantity of reducing solvent in a conventional scale tank equipped with a water cooled solvent reflux condenser and further provided with a mechanical agitator.

Three thousand two hundred and twenty pounds of the superbodied oil produced in accordance with the foregoing procedure was thinned by pumping it at a temperature of 450° F. from the bodying kettle into a stainless steel thin-down tank equipped with a water-cooled reflux condenser and containing 96.6 pounds of the monoethyl ether of ethylene glycol. The mixture of oil and solvent was mechanically agitated for one hour using a motor driven turbo agitator. At the same time recirculation by pumping the oil and solvent mixture from the bottom of the thin-down tank into the top was provided to further assure a thorough blending, at an elevated temperature, of the oil with the solvent.

At the close of this mixing cycle the batch in the thin-down tank was allowed to rest, with only natural convection cooling being provided through the wall of the thin-down tank to a temperature of 180° F., over a period of 11 hours. During this long cooling cycle the viscosity of the solvent-oil solution became 3 minutes and 30 seconds.

At this point 2400 pounds of the solution was pumped into a stainless steel air-blowing vessel equipped with a motor-driven turbo agitator, a water-cooled reflux condenser, a steam-heating or water-cooling coil, and a perforated coil for passing air into and through the oil while mechanically agitating it to further break up the air bubbles and to lengthen the path of travel by the air in the interest of creating a more extensive air-oil interface. As indicated above, instead of pumping to a separate tank, the aeration could as well have been carried out in the thermal polymerization reactor such as shown in FIG. 1.

This aeration was conducted after cooling the reduced oil further to 170° F. during the time of pumping it from the thin-down tank into the blowing tank with a further lowering of the temperature an additional two degrees to the above-mentioned 170° F., employing for this purpose water in the cooling coil of the blowing tank.

Aeration was conducted at temperatures ranging between 170° F. to 180° F. for 35 hours at which point the oil had become free of solvent as a consequence of losses of the solvent to the atmosphere through air entrainment despite the passage of the discharged air through the reflux condenser. This solvent-free oil, in which was dispersed a considerable amount of entrapped air as fine bubbles, had a viscosity of 17 minutes, after removing the entrapped air from the test sample.

During the elapsed time from the taking of the sample, and its centrifuging for a removal of its entrapped air, and a determination of the viscosity of the air-free oil, the air-blowing had been continued. As soon as the 17 minute viscosity reading was obtained in the test the blowing of the air through the oil was stopped. The amount of

the elapsed time from the taking of the sample until cessation of the blowing with air was 45 minutes. A sample taken at this point had a viscosity of 18 minutes and 45 seconds. At this time 71.3 pounds of monoethyl ether of ethylene glycol and 166.3 pounds of V.M. & P. naphtha were added to the oxidized oil in the blowing tank. This mixture was mechanically stirred and recirculated by pumping until a thorough and complete solution occurred. The stirring and recirculating was stopped and the batch was allowed to stand in the blowing tank for two hours and thirty minutes to achieve a removal of most of the entrapped air through its rising to the surface. At this point a sample was taken for a reduced oil viscosity determination and this viscosity was found to be 3 minutes and 40 seconds. Relating this viscosity to a chart, obtained through the determination of the viscosities of similar oxidized oils at various unreduced viscosities, enabled a finding, through this reference, of an unreduced oil viscosity of 20 minutes, based upon the reduced oil viscosity of 3 minutes and 40 seconds. This increase in the viscosity of the oil is due to its further oxidation by the entrapped air bubbles.

The characteristics of the reduced, oxidized oil were:

|                             |       |
|-----------------------------|-------|
| Viscosity -----             | 3'40" |
| Acid value -----            | 4.6   |
| Color (Gardner, 1933) ----- | 11    |

In a second example of the production of a high polymer linseed oil having a viscosity of from 50 to 60 minutes, Gardner-Holdt, the following procedure is followed. The cooking kettle, such as the kettle shown in FIG. 1 in diagrammatic form, is charged with 3700 pounds of an alkali refined, refrigerated linseed oil. The batch is agitated with carbon dioxide, and vacuum applied to the extent of about 28" of mercury. Heat is applied for a period of about 2.75 hours until the temperature reaches about 450° F. At this point, steam is introduced into the body of the oil through a plural vent pipe located at the bottom of the tank, the rate of steam flow through the body of oil being determined by the tendency for loss of oil through the vapor vent at the top of the kettle, the rate of flow being regulated to prevent such loss. Carbon dioxide is blown through the body of the oil simultaneously with the steam. The vacuum is held at 28" of mercury, and the temperature elevated to about 575° F. The heat is held at this point with a minimum rate of heat input into the apparatus. The temperature reaches about 575° F. in about 65 minutes time and is held at this temperature until a viscosity of from 40 to 50 seconds is obtained. This takes a period of time of about 7 hours and 10 minutes.

At the 40 second viscosity, all heat input is terminated, and the vacuum released. The vacuum pump is kept operating, and the steam blow is reduced, if necessary, to maintain proper level of the oil in the kettle. At this point, 10.75 pounds of a mineral spirits solution of 24% lead isodecanoate is added very slowly and carefully. Immediately thereafter, 16.25 pounds of a lithium naphthenate dispersion in water having a lithium metal content of from 1.2-1.6% lithium is added. This solution contains some water and will tend to crackle slightly on mixing with the hot oil. After the addition has been completed, the tank is again sealed, and the vacuum slowly and carefully reapplied to 28" of vacuum. Maximum steam blow is again obtained, and the batch held under these conditions for a viscosity of from 7 to 8 minutes. At this point, the temperature is dropped to about 550° F. It has been predetermined for this particular oil that viscosities in this range are critical beyond which the thermal homopolymerization of the linseed oil will become uncontrollable at 575° F. The heat is now allowed to fade to about 550° F. by cutting off one of the heat input burners. Cooling water may be introduced through the cooling coil intermittently, if necessary. About 30 minutes later, the temperature has achieved 550° F., and the

viscosity is determined to be about 9 minutes, Gardner-Holdt. All heat input is terminated and the vacuum released. The vacuum pump is maintained operative in order to provide a slight negative pressure so fumes from the kettle go through the pump. Foaming caused by the steam should have subsided at this viscosity. At this point, there are slowly added 36 pounds of glycerin, or other polyhydric alcohol containing from 3 to 10 carbon atoms and at least 3 hydroxyl groups such as, pentaerythritol, dipentaerythritol, trimethanol ethane, trimethylolpropane, triethanol ethane, sorbitol, mannitol, etc. The addition of the polyhydric alcohol should be done over a period of about 30 minutes. When the addition has been completed, the kettle is again closed, and the 28" vacuum slowly and carefully reapplied.

After the body of the oil has reached about 14 minutes, Gardner-Holdt, samples are then taken every 15 minutes. About 60 minutes after the attainment of the 9 minute viscosity, the viscosity is found to have increased to 24 minutes. At this point the burner flame is reduced and heat allowed to fade to about 500° F. while maximum steam blow and 28" mercury vacuum are maintained. These conditions are maintained until the body of the oil has reached about 45 minutes, Gardner-Holdt, occupying a time period of an additional 90 minutes. The heat is maintained at about 500° F. until the viscosity has reached about 51 minutes.

At this point, the batch is checked by putting cold water through the kettle cooling coil and dropping the temperature sharply to 450° F. After an additional 40 minutes, the viscosity of the oil is 54 minutes, Gardner-Holdt, and the temperature of the batch is 450° F.

Preparation is then made to drop the oil into a thindown tank, the transfer line from the varnish kettle to the thindown tank being preheated with steam, and the reflux condenser above the thin-down tank cooled with water.

The thinner into which the oil is dropped may consist of approximately 100 pounds of a polar solvent which desirably contains free hydroxyl and an ether or a ketone group. These polar solvents have an unusual effect upon superbodied oils which is not clearly understood but which is quite important in the production of stable emulsified superbodied oils whether these oils are merely superbodied or the pre-oxidized superbodied oils.

Specific examples of such polar solvents include aliphatic keto-hydroxyl compounds and ether-hydroxyl compounds. A principal class of materials includes the lower alkyl monoethers of alkylene glycols for example the methyl, ethyl, propyl, isopropyl ethers of ethylene glycol, trimethylene glycol, tetramethylene glycol, pentamethylene glycol, hexamethylene glycol, diethylene glycol, etc. Specific examples of keto-alcohols include methylene hydroxy ethyl ketone, hydroxy propyl methyl ketone, hydroxy butyl methyl ketone, hydroxy decyl methyl ketone, hydroxy ethyl ethyl ketone, hydroxy ethyl propyl ketone, hydroxy ethyl butyl ketone, etc. For most purposes, the methyl, ethyl, and propyl or isopropyl mono ethers of ethylene glycol and diethylene glycol are preferred.

Some kind of interaction takes place between oxygen containing solvent materials and the superbodied oil to effect a reduction in the body of the oil which surpasses what would be expected from normal dilution effect. Nevertheless, whether an emulsion is made from the superbodied oil at this point, or whether the oil at this point is subjected to the pre-oxidation procedure as above outlined, there is observed a marked improvement in the nature of the emulsion which is obtained. This is far more suitable, and the particle size of the oil droplets in the emulsion is so fine that present means for determining particle size are ineffective. These particles are in the sub-micron range. Not only is there an improvement in the stability in the emulsion but there is also noted a marked improvement in the process of producing the emulsion by an inversion technique as described in my

previous application Ser. No. 329,196. It has also been noted further that the treatment of the superbodied oils with the polar solvents in the amount of from 2% to 5% by weight of the oil following the bodying step effects an improvement in emulsion stability and emulsion formation regardless of whether the superbodied oil condition is obtained by the precise thermal bodying steps as set forth above or by other conventional superbodied procedures such as the Arvin procedure described in his Patent 2,607,784.

Returning to the second example, the resultant superbodied oil may be treated in precisely the same fashion as set forth above to produce a preoxidized superbodied oil. The resultant material has a solvent reduced viscosity of 3 minutes and 50 seconds, and acid value of 4.9, and a color, Gardner of 10.

As indicated above, the apparatus used for the pre-oxidation step of this process may be the original bodying apparatus such as shown in FIG. 1 utilizing the main sparge line connected to a pressurized air source instead of a steam source. The same perforated ring disposed in the bottom of the reactor vessel is convenient for distributing the air through the mass. It is preferable to agitate the batch with the agitating blades for the purpose of maximizing insofar as possible the oil-air interface.

The blowing operation is carried out at a temperature as indicated above in the range of from 150° F. to 200° F., and preferably in the range of from 170° F. to 180° F. The time required for the oxidation phase of the polymerization may range from 25 to 60 hours, and for most purposes it will be found satisfactory to carry out this oxidation for a period of between 30 and 40 hours. The resultant pre-oxidized superbodied oil will be found to have a viscosity within the range of from about 20 minutes to about 75 minutes. This product because of the conditions of the oxidation phase is now a solvent free material and is immediately reduced following the attainment of the desired viscosity with a solution which is composed of a polar oxygen-containing solvent and a hydrocarbon solvent. A particularly preferred example of such solvent is three parts of ethyl Cellosolve, seven parts of light mineral spirits based on 100 parts by weight of the oil to thin the oil and to interfere with any tendencies toward after-bodying in the holding vessel.

The resultant pre-oxidized superbodied oils may now be emulsified as described in the previous copending applications.

Other modes of applying the principle of this invention may be employed instead of those specifically set forth above, changes being made as regards the details herein disclosed, provided the elements set forth in any of the following claims, or the equivalent of such be employed.

It is, therefore, particularly pointed out and distinctly claimed as the invention:

1. In a process for making a superbodied unsaturated fatty oil free from gel particles and false body, and having a viscosity in the range of from 20 minutes to 75 minutes, Gardner-Holdt, which process includes the steps of:

- (a) heating the body of said oil under sub-atmospheric pressure to the temperature of incipient polymerization for said oil;
- (b) contacting said body of oil with water vapor at said temperature;
- (c) increasing the temperature of said body of oil to a maximum temperature not in excess of about 615° F. to initiate and sustain thermal polymerization of the oil while continuously contacting the body of oil with water vapor;
- (d) maintaining the body of oil under thermal polymerization conditions until the viscosity of the oil

reaches a maximum viscosity in the range of from about 20 minutes to about 75 minutes, Gardner-Holdt, while continuously contacting the body of oil with water vapor;

- 5 (e) discontinuing the contacting of said body of oil with water vapor; and
  - (f) checking the oil by rapidly dropping the temperature to below that required to sustain thermal polymerization;
- 10 the improvement which comprises:

- (g) oxidizing with an oxygen-containing gas the thermally polymerized oil in bulk at a temperature of from about 150° F. to about 200° F. for a period of from 25 to 60 hours.

15 2. The process of claim 1 in which the unsaturated fatty oil is linseed oil.

3. The process of claim 2 in which the linseed oil is an alkali refined linseed oil.

20 4. The process of claim 1 in which the unsaturated fatty oil is a mixture of alkali refined linseed oil, dehydrated castor oil, and soya bean oil in a weight ratio of 2:1:2.

25 5. In a process for making a superbodied alkali refined linseed oil free from gel particles and false body, and having a viscosity in the range of from 20 minutes to 75 minutes, Gardner-Holdt, said process including the steps of:

- (a) heating a body of said oil under a pressure of from about 5 mm. to about 150 mm. of Hg to a temperature of about 450° F. while blowing the body of oil with an inert gas;
- (b) after the temperature of the oil is at about 450° F. blowing the body of oil with steam;
- (c) heating said body of oil to a maximum temperature of about 580° F. in about 60 minutes time while continuing to blow the oil with steam;
- (d) maintaining said conditions of temperature pressure and steam blowing until an oil viscosity of about 7-10 minutes, Gardner-Holdt, is reached;
- (e) lowering the temperature to about 500 to about 560° F. and continuing the pressure and steam blowing until the viscosity in the range of from 20 minutes to 75 minutes, Gardner-Holdt, is achieved;
- (f) quickly cooling the batch to a temperature below about 475° F.;

45 the improvement which comprises:

- (g) thinning the resultant heat bodied oil with a solvent to reduce the viscosity of the heat bodied oil-solvent mixture to about 2 minutes to about 10 minutes, Gardner-Holdt;

(h) cooling the oil-solvent mixture to a temperature of from between 150 to 200° F.;

(i) blowing the oil-solvent mixture at this temperature with an oxygen-containing gas for a period of from 25 to 60 hours.

60 6. A process in accordance with claim 5 in which the solvent is ethyl Cellosolve (the mono-ethyl ether of ethylene glycol).

7. A process in accordance with claim 5 in which the oxygen-containing gas is air.

#### References Cited

##### UNITED STATES PATENTS

|    |           |        |          |       |           |
|----|-----------|--------|----------|-------|-----------|
| 65 | 2,248,964 | 7/1941 | Corkery  | ----- | 260—406   |
|    | 2,248,965 | 7/1941 | Corkery  | ----- | 260—407   |
|    | 2,754,308 | 7/1956 | Grummitt | ----- | 260—407 X |
|    | 2,822,371 | 2/1958 | Nichols  | ----- | 260—407 X |

70 NICHOLAS S. RIZZO, Primary Examiner.

F. A. MIKA, Assistant Examiner.